

# UNITED STATES PATENT OFFICE.

JEROME W. FRANK, OF NEW YORK, N. Y., ASSIGNOR TO STANDARD VARNISH WORKS, OF NEW YORK, N. Y., A CORPORATION OF NEW YORK.

## SOLID INSULATING COMPOUND.

No. 895,738.

Specification of Letters Patent. Patented Aug. 11, 1908.

Application filed June 28, 1907. Serial No. 381,359.

*To all whom it may concern:*

Be it known that I, JEROME W. FRANK, a citizen of the United States, and resident of the borough of Manhattan, in the city and State of New York, have invented a new and useful Improvement in Solid Insulating Compounds, of which the following is a specification.

My invention relates to an insulating compound and particularly to an insulating compound capable of use in insulating transformer coils intended for use immersed in oil.

The object is to provide a compound having good insulating properties and a high degree of penetration and an added function of retaining its ability to be liquefied after repeated heatings.

My invention consists of a solid insulating compound composed of castor oil, a resinous gum from a coniferous tree, such, for instance, as colophony, a fossil gum, such for instance, as the New Zealand gum known commercially as gum kauri, or the Dutch East India copal gums known commercially as Manila gum and Pontiniac gum.

The several ingredients may be practically combined in the following proportions:—100 pounds gum kauri, 25 pounds colophony, 5 gallons castor oil.

The gum kauri and colophony are first melted and then the castor oil is added and the mixture boiled until the ingredients are thoroughly united. After cooling, this compound is ready for use.

The proportions may be varied within reasonable limits to suit special requirements.

In stating the formula I have taken gum kauri, colophony and castor oil as samples of the various classes of ingredients which I

have mentioned, it being understood that I do not limit myself to the specific types mentioned. The material thus formed after being liquefied under heat is especially well adapted for impregnating in vacuum fabric-covered wires wound into coils of various forms for the purpose of filling the interstices and insulating said coils and providing a filler and coating impervious to mineral oil.

It is an oil resisting insulating filler and covering suitable for insulating transformer coils which operate in a cooling bath of oil, the colophony serving to prevent the compound after repeated heatings from becoming a pasty mass without penetrating properties and incapable of being liquefied below a temperature in excess of that which would destroy the fabric covering of the wires in the coils and moreover render the compound valueless as an insulator and filler for transformer coils.

What I claim is:—

1. A solid insulating compound composed of castor oil, a fossil gum and a resinous gum from a coniferous tree combined in the proportions substantially as specified.

2. A solid insulating compound composed of castor oil, gum kauri and colophony combined in the proportions substantially as specified.

In testimony, that I claim the foregoing as my invention, I have signed my name in presence of two witnesses, this 22nd day of June, 1907.

JEROME W. FRANK.

Witnesses:

W. H. STETT,  
R. CRISSON.